

## UNITED STATES PATENT OFFICE

2,051,937

## STEEL-ALLOY RIVET

Herbert Buchholtz, Dortmund, Germany, assignor to the firm Vereinigte Stahlwerke Aktiengesellschaft, Dusseldorf, Germany

No Drawing. Application January 10, 1934,  
Serial No. 706,149. In Germany January 21,  
1933

1 Claim. (Cl. 85—37)

This invention relates to an improvement of rivets of an ingot steel which is produced by melting in the usual manner and is free from slag content.

- 5 Highly stressed structures such as bridges made from steel which is known in Germany as "St 52" (that is, a steel with a tensile strength of over 50, and a yield point of at least 36 kg. per sq. mm. with good ductility and tenacity) require for connecting the structural elements, rivets with a shearing strength corresponding to that of the material to be united, in order that the loading capacity of the steel shall be fully and economically utilized. According to existing experience, this object is achieved—though only by putting up with other drawbacks—by selecting a rivet steel of similar composition to the St 52 steel employed in each case, but having a strength of only about 48 kg. per sq. mm.
- 20 Applicant's researches have now revealed that the alloyed rivet steels compounded in accordance with the above considerations have a relatively low binding power during the riveting process. If, for example, nickel or manganese steels 25 be employed as such alloyed rivet steels, the riveted joints exhibit a very low resistance to slip, owing to the low binding power of said alloyed rivet steels, so that the danger arises of the joints soon working loose, especially when alternating stresses occur. If, on the other hand, unalloyed rivet steels be employed, with a tensile strength of 30 34 or 42 kg. per sq. mm., then, although the binding power is satisfactorily high, the shearing strength, in the case of St 34 steel, is lower than that of the plate material, whilst in the case of 35 rivets of St 42 steel the shearing strength is not always satisfactory and the tenacity is lower than in alloyed rivets.

According to the present invention, the various 40 conflicting requirements that must thus be imposed on a high-grade rivet steel for highly-stressed structures can be fulfilled by selecting a low carbon and manganese content and such alloying components that do not (or only to a slight 45 degree) lower the temperature at which the iron is transferred from the so-called  $\gamma$ -condition into the so-called  $\alpha$ -condition. Alloying components of said kind are silicon, molybdenum, copper and vanadium. By using said alloying additions in 50 the amounts and combinations hereinafter specified it is possible to obtain valuable rivet steels with a relatively high temperature of the  $\gamma/\alpha$  transformation which simultaneously possess a low hysteresis and a raised yield point in the 55 range between 450 and 650°C.

The effect of a high transformation point is that the contraction which the rivet is left to undergo after the riveting operation is completed, is not disturbed by any transformation. A low hysteresis of transformation prevents the 5 production of a hardening structure during the accelerated cooling of the hammered rivet by the steel masses surrounding it. The formation of a hardening structure causes, as is known, an increase of volume and an insufficient toughness 10 and would thus diminish the binding power and the tenacity of the hammered rivet. The high limit of thermal ductility aimed at by the present invention enables to obtain a high binding power at higher temperatures as well as after the rivet 15 has been cooled. Therefore, according to the invention the preliminarily hammered rivet steel is chosen in such a manner that by the riveting process which is carried out under otherwise normal conditions, rivets are produced which possess 20 not only the same values of yielding limit, tensile strength and elongation as the surrounding plate material, but which also possess a high binding power, a high shearing strength and tenacity.

The rivet according to the invention consists 25 of a steel containing carbon from trace to 0.13%, manganese from trace to 0.5%, silicon between 0.35 and less than 0.5%, and copper from trace to 1%. A rivet composed in such a manner is adapted, after the mechanical treatment of riveting, to assume a tensile strength of at least 50 kilograms per square millimeter, a yield limit of 30 at least 40 kilograms per square millimeter and a notch-bar tenacity of at least 10 kilograms per square millimeter.

The following composition, strength properties 35 are given, by way of example, together with the binding power of 25 mm. rivets after hammering, for characterizing the essential properties of an alloyed rivet steel produced according to the 40 present invention.

## Composition

| O    | Si   | Mn   | Cu   |                                           |
|------|------|------|------|-------------------------------------------|
| 0.09 | 0.48 | 0.45 | 0.42 | Remainder iron with the usual impurities. |

45

Bundles of five 25 mm. plates were riveted with 50 rivets of said steel, by means of a pneumatic hammer (air pressure 6.5 atmospheres) in about 18 seconds. The binding power of the hammered rivets was determined by the method of C. Bach and found to lie between 32 and 41 kg. per sq. 55

mm., with a mean of 37 kg. per sq. mm. The strength properties of the hammered rivets were ascertained from tensile specimens 10 mm. in diameter and 50 mm. measurement length, the shearing strength with doubly notched test pieces, the notched-bar tenacity on test pieces measuring 10 x 10 x 60 mm. with a rounded notch 3 mm. in depth and 2 mm. in diameter.

The mean results are given below:

| 10 | Yield point mkg. | Tensile strength per sq. mm. | Elongation percent | Constriction percent | Shearing strength kgs. per sq. mm. | Notched-bar tenacity per sq. cm. |
|----|------------------|------------------------------|--------------------|----------------------|------------------------------------|----------------------------------|
| 15 | 41               | 54                           | 29                 | 63                   | 44                                 | 22                               |

The results of these tests show the hammered rivets to be a material of high yield point and shearing strength, and of medium tensile strength accompanied by high ductility and notched-bar tenacity. The binding power, with the mean value 37 kg. per sq. mm., is situated near the yield point and is about 40 to 50% higher than in rivets of St 34 steel, riveted under the same conditions. Other suitable rivet steels produced according to the present invention had the following composition:

| 30 | C                 | Si                | Mn                | Cu                |
|----|-------------------|-------------------|-------------------|-------------------|
| 35 | Percent 0.08-0.13 | Percent 0.35-0.49 | Percent 0.35-0.45 | Percent 0.25-0.40 |

The high binding power of the rivets also in-

fluences of course, the resistance of riveted joints to slip. Thus, in the micro-measurement test of double-row riveted joints of steel with a tensile strength of 55 kg. per sq. mm., the rivets of the present invention gave a resistance of 14 to 16 kg. per sq. mm. to slip, whereas with rivets of unalloyed carbon steel with approximately 0.08% C, the resistance was only 7 to 8 kg. per sq. mm.

Permanent stress tests of rivet joints made with rivets produced according to the present invention, under increasing permanent stress, showed an original strength 25% greater than joints made, under otherwise equal conditions, with rivets of soft carbon steel. If hard rivets of, for example, 3% nickel steel were employed in place of the soft rivets of carbon steel, the binding power and original strength would be substantially lower than with rivets produced according to the present invention.

For the workshop, the low sensitiveness to overheating, and the relatively small formation of scale, of the rivet steel according to the present invention, also proved a considerable advantage.

What I claim and desire to secure by Letters Patent of the United States is:

A rivet of an ingot steel alloy containing carbon from trace to 0.13%, manganese from trace to 0.5%, silicon 0.35 to less than 0.50% and copper from trace to 1% and the balance substantially iron, said rivet being adapted, after the mechanical treatment of riveting, to assume the following properties, tensile strength at least 50 kg. per square mm., yield point at least 40 kg. per square mm. and notch-bar tenacity at least 10 mkg. per square cm.

HERBERT BUCHHOLTZ.